

## UNITED STATES PATENT OFFICE

PAUL KARRER, OF ZURICH, SWITZERLAND, ASSIGNOR TO HEBERLEIN & CO., A. G., OF WATTWIL, SWITZERLAND, A CORPORATION OF SWITZERLAND

## TREATMENT OF CELLULOSE FOR CHANGING ITS ACTIVITY TOWARD DYESTUFFS

No Drawing. Application filed May 14, 1929, Serial No. 363,103, and in Germany May 23, 1928.

This invention relates to the treatment of cellulose for changing its activity toward dyestuffs. It is particularly directed to acetylizing cellulose so that it is immunized against substantive dyes. It also relates to a product resulting from such treatment.

In the treatment of cellulose fibres with a mixture of acetic anhydride, glacial acetic acid and a catalyst such as sulphuric acid, zinc chloride, formic acid, etc., there occurs an acetylation of the cellulose accompanied by a gradual disintegration of the fibre and finally complete solution of the acetylated cellulose in the mixture. By interrupting the process after a certain period it is, of course, possible to obtain partially acetylated fibres which still retain more or less of their original structure. (Cf. British Patent 280,493.) Such fibres show some immunity to substantive coloring matters.

It has been found in accordance with the present invention that the limits between complete solution when the fibre no longer exists and acetylation to a point where the fibres are not destroyed but possess immunity to substantive dyestuffs, lie close together. It is, therefore, extraordinarily easy for too much acetylation to occur, and if it does a corresponding weakening of the fibre occurs at the same time. In addition when acetylation continues longer than necessary the immunity of the fibre to the dye lessens or disappears. Apparently this is so because acetylation occurs only on the surface of the fibre and the acetylated layer, first formed by further action of the acetyling mixture is dissolved.

The object of the present invention accordingly is to provide a simple, inexpensive process of the kind described by which the degree of acetylation of a fibre may be controlled to produce a fibre having immunity to substantive dyestuffs while substantially preserving the structure and other desirable characteristics of the fibre. Another object of the invention is to provide a product of the kind mentioned having the desired immunity to substantive dyestuffs and possessing the strength and other desirable characteristics of the original fibre. Further

objects and advantages of the invention will more fully appear in the following description of some preferred methods of carrying out the invention.

I have made the unexpected observation, in accordance with this invention, that trioxymethylene, formaldehyde, polyoxymethylene or other polymers or derivatives of formaldehyde or compounds which liberate formaldehyde under the reaction conditions, designated broadly herein as "formaldehyde equalizers", when added to an acetylizing mixture of glacial acetic acid, acetic acid anhydride and a catalyst (for example, sulphuric acid or zinc chloride), act as equalizers of acetylation. They very extraordinarily and in great measure slow down the weakening or solution of the cotton threads in the acetylizing fluid. By the term equalizer as used above, I mean that the reagent acts to provide a substantially uniform effect on the surface treated with the acetylizing agent. This effect is a partial acetylation. From my observations the interior of the fiber remains unchanged while the exterior surface is given a skin or coating of acetylated cellulose. For example, cotton which, at room temperature, is dissolved in an ordinary acetylizing mixture within 48 hours is completely intact even after 6 to 8 days when treated with the same acetylizing mixture modified by a formaldehyde equalizer. The acetylizing itself through the addition of formaldehyde or the like is in no way interfered with. Furthermore, one obtains fibres which, compared with those acetylated without formaldehyde, or the like, show a higher degree of immunity to dyestuffs. Through careful warming the reaction can be aided and hastened. The process possesses important technical advantages.

## Examples

(1) In a mixture of ten parts glacial acetic acid, eight parts acetic acid anhydride, one part of zinc chloride and two parts of p-formaldehyde, a portion of cotton yarn is immersed at room temperature, about 18° C. and kept there. After two days the treated yarn has a suitable immunity against sub-

- stantive dyestuffs which, in the course of the next few days increases, and attains after 100 to 170 hours, a high degree of immunity. By gradually warming this mixture to 40° C., the reaction is hastened and high degree of immunity can be obtained in 24-48 hours while preserving the other desirable characteristics obtained at lower temperatures.
- (2) In a mixture of 10 parts of glacial acetic acid, 12 parts of acetic acid anhydride, 1 part of zinc chloride and 4 parts of a solution containing 40% of formaldehyde, a portion of cotton yarn is immersed at room temperature of about 18° C. and kept there.
- 15 After 2 days the treated yarn is suitably immunized against substantive dyestuffs which in the course of the next 2 days increases and obtains after 100 to 150 hours a high degree of immunity.
- 20 (3) In a mixture of 8 parts of glacial acetic acid, 7 parts of acetic acid anhydride and 2 parts of zinc chloride, and 1.5 parts of trioxy-methylene, a portion of cotton yarn is immersed at room temperature of about 18° C. and kept there. After 2 days the treated yarn is suitably immunized against substantive dyestuffs which in the course of the next 4 days increases and obtains after 150 to 170 hours a high degree of immunity.
- 25 39 In place of the equalizers mentioned in these examples, other formaldehyde modifications may be employed including polyoxymethylene, other polymers, derivatives of formaldehyde or other combinations which produce formaldehyde in the acetylizing mixture. In place of zinc chloride sulphuric acid may be used as a catalyst.
- 40 Thus while I have described my improvement in detail and with respect to certain preferred forms, I do not desire to be limited to such details or forms since, as will be noticed by those skilled in the art, after understanding my invention many changes and modifications may be made and the invention embodied in widely different forms without departing from the spirit and scope thereof in its broader aspects, and I desire to cover all modifications, forms and improvements coming within the scope of any one or 50 more of the appended claims.
- 45 Having thus described my invention what I claim as new and desire to secure by Letters Patent is:
- 55 1. A process of the kind described which comprises treating a substance containing cellulose with an acetylizing agent in the presence of a formaldehyde equalizer and acetylizing the cellulose-containing substance until it has a partial acetylation sufficient 60 to give it immunity to substantive dyestuffs.
- 65 2. A process of the kind described which comprises treating cotton fibre with an acetylizing agent containing glacial acetic acid, acetic acid anhydride, a catalyst and a formaldehyde equalizer and acetylizing the
- 70 fibre until it has a partial surface acetylation sufficient to give it immunity to substantive dyestuffs.
- 75 3. A process of the kind described which comprises subjecting cellulose fibre to a bath containing an acetylizing agent and a formaldehyde equalizer, and acetylizing said fibre until it has a partial surface acetylation giving it immunity to substantive dyestuffs.
- 80 4. A process of the kind described which comprises immersing cellulose in a bath containing glacial acetic acid, acetic acid anhydride, a catalyst and a formaldehyde equalizer and acetylizing said cellulose until it has a partial surface acetylation giving it immunity to substantive dyestuffs.
- 85 5. A process of the kind described which comprises subjecting cellulose fibre to a bath containing glacial acetic acid, acetic acid anhydride, a catalyst and p-formaldehyde and acetylizing said fibre until it has an acetylated surface giving it immunity to substantive dyestuffs.
- 90 6. A process of the kind described which comprises subjecting cotton fibre to the acetylizing action of glacial acetic acid, acetic acid anhydride, zinc chloride and p-formaldehyde and continuing the acetylation at about room temperature for 100 or more hours.
- 95 In testimony whereof I have signed my name to this specification.
- PAUL KARRER.
- 100
- 105
- 110
- 115
- 120
- 125
- 130